# EUROPEAN PATENT SPECIFICATION

(11) **EP 1 601 472 B1**
(45) Date of publication and mention of the grant of the patent: **19.03.2008**
(21) Application number: 04713921.7
(22) Date of filing: 24.02.2004
(51) Int. Cl.: B08B 9/02, B08B 9/027, C22F 1/08

(54) **METHOD FOR TREATING THE INNER SURFACE OF A TUBE**
VERFAHREN ZUR BEHANDLUNG DER INNENFLÄCHEN EINES ROHRS
PROCEDE SERVANT A TRAITER LA SURFACE INTERIEURE D'UN TUBE

(30) Priority: 07.03.2003 FI 20030344
(43) Date of publication of application: 07.12.2005
(73) Proprietor: Outokumpu Oyj, 02200 Espoo (FI)
(72) Inventor: HARJU, Terho, FIN-28100 Pori (FI); SALMINEN, Aleksi, FIN-28800 Pori (FI); NORÈN, Timo, FIN-28200Pori (FI)
(74) Representative: Zipse Habersack Kritzenberger
(86) International application number: PCT/FI2004/000086
(87) International publication number: WO 2004/078372

(56) References cited:
- EP-A1- 0 647 723
- FR-A1- 2 623 110
- GB-A- 1 461 961
- JP-A- 8 213 812
- US-A- 4 445 350

## Description

The invention relates to a method according to claim 1 for manufacturing a copper or copper alloy tube. In particular, the invention relates to a cleaning treatment carried out on the inner surface of an extruded tube before the tube is worked to its final size.

When extruding seamless metal tubes, such as copper tubes, a solid metal billet is by means of a mandrel worked to the form of a tube. When lubricating the mandrel surface, there are used for instance graphite-based materials, the contents of which may be harmful in the further processing of the tubes. Hot extruded tube billets, i.e. extruded tubes, are thereafter drawn to their final size. After extrusion, the extruded tubes can also be worked to their final size by rolling.

In the drawing steps, there are generally used oil-based lubricating materials, which may leave carbon-bearing impurities on the inner surface of the tube. It is well known that the lengthwise grooves created on the inner surface of an extruded tube may form fold-backs in the tube drawing steps. Lubricating materials used both in the extrusion and in the drawing steps can remain in said fold-backs. It has generally been found out that the carbon content of the inner surfaces cannot necessarily be adjusted to the required level by means of known degreasing washings or other solvent treatments, which causes problems for instance in the metal coating of the inner surface. Especially problems have been detected for example in the adhesion of a tin coating. All in all, it would be important to affect the properties of the inner surface already at the beginning of the tube manufacturing process, in order to even out the grooves created in the tube inner surface already at the extruding step, and to remove all graphite residues therefrom.

From the publication EP 335999 there is known a cleaning method for cleaning a copper tube manufactured by drawing. The method relates to the removal of lubricant greases after the drawing by means of sand blasting.

From the FI patent application 20001467 (corresponding to EP-A-1 167 563) there is known a method for coating the inner surface of copper or copper alloy tubes by a protecting film, particularly tin film, in which method the coating step is preceded by a mechanical treatment of the surface to be coated.

Other methods and apparatus for treating the inner surface of extruded copper tubes are known from documents JP-A-08 213 812 and EP-A-0 647 723. The object of the present invention is to introduce a novel method for manufacturing copper or copper alloy tubes, in which method the inner surface of the extruded tube is subjected to a cleaning treatment before the tube is worked to its final size.

The object of the invention is attained by the combination of features of claim 1. Preferred embodiments of the invention are characterized by what is set forth in the dependent claims.

Remarkable advantages are achieved by means of the method according to the invention. The invention relates to a method for manufacturing copper or copper alloy tube, which method includes an extrusion step and at least one working step for working the tube to its final size, and according to which method, the tube inner surface is subjected to a cleaning treatment, so that the cleaning treatment is performed on the inner surface of the extruded tube before the tube is worked to its final size. Here a tube means an end product. By means of the invention, it is possible to essentially improve the quality of the inner surface of metal tubes, such as copper tubes. According to a preferred embodiment of the invention, a tube is worked to its final size by drawing an extruded tube at least in one step. In this case the cleaning treatment is carried out essentially between the extrusion step and the drawing step. According to a preferred embodiment of the invention, the tube is worked to its final size by rolling the extruded tube at least in one step. Now the cleaning treatment is carried out essentially between the extrusion step and the rolling step. When the inner surface of a hot extruded tube billet, i.e. an extruded tube, is cleaned before working the tube to its final size, there is achieved a tube end product with an excellent carbon content.

According to a preferred embodiment of the invention, the cleaning treatment is carried out mechanically. One method according to the invention is that the cleaning treatment is carried out by treating the inner surface of the extruded tube with a cleaning device that is made of an essentially harder material than the inner surface. Thus also graphite-based impurities are advantageously removed. According to an embodiment of the invention, the employed cleaning device is a steel brush. In this fashion, impurities are advantageously detached from the inner surface. According to an embodiment of the invention, the cleaning device is moved along the inner surface of the extruded tube by means of magnets. According to another embodiment, the cleaning device is moved along the inner surface of the extruded tube by means of an elongate shaft. According to an embodiment, in the cleaning treatment the extruded tube is moved with respect to the cleaning device. One way according to the invention is that the cleaning treatment is carried out by grain blasting, such as sand blasting. By treating the inner surface of the extruded tube created in the extrusion step, i.e. the so-called first inner surface of the tube, mechanically, the grooves created in the tube surface during the extrusion are evened out, and the graphite residues are removed. Consequently, it is not anymore - neither in the extrusion step nor in any further processing steps - necessary to take into account the possible circulation of graphite and carbon contaminations to the end product, but it is possible to concentrate on other matters that are important for the process.

According to the invention, after a mechanical cleaning treatment, the inner surfaces of the extruded tube are blasted by gas. Another way according to the invention is that after a mechanical cleaning treatment, the inner surfaces of the extruded tube are washed by liquid. According to an embodiment of the invention, the tube is subjected to a coating treatment after working the tube to its final size.

An extruded tube treated according to the invention makes it easier to perform further processing, such as metal coating. In addition, it is possible to achieve on the surface such carbon contents that comply to the regulations. By applying the method, the carbon content of the inner surfaces of tube end products can be controlled better than in the prior art. Moreover, savings in the expenses are achieved both in employed work and materials, as well as in the pretreatment steps that require metal coating. By cleaning the initial tube that feeds the whole production process, all further processes up to the end product are remarkably facilitated as regards the requirements for surface cleanness.

The invention is described in more detail below with reference to the appended example.

### Example

In the example, there is observed the processing of a tube that in the final measures has an outer diameter of 54 millimeters, from an extruded tube by applying the method according to the invention. The example describes how the inner surface of the extruded tube was cleaned, and how the cleaned extruded tube behaved in test drawings in comparison with a regular uncleaned extruded tube. After test drawings and washings, the inner surface was observed by various different surface test methods. In addition, there was observed the metallic coatability of tubes manufactured according to the invention.

In the extrusion step, all graphite residues and grooves left on the inner surface of the extruded tubes were removed by a cleaning device made of steel. The graphite ingredients were detached by manually rotating the cleaning device along the inner surfaces of the extruded tubes, whereafter the extruded tubes were blasted by pressurized air. The mechanically cleaned extruded tubes were transported to drawing. As a result, it was found out that in the first drawing, a cleaned extruded tube requires a drawing force that is about 5% higher than with an uncleaned extruded tube. After the first drawing, drawing behavior does not differ from the drawing behavior of regular uncleaned extruded tubes.

The qualities of the inner surfaces of a regular uncleaned extruded tube and of a mechanically cleaned extruded tube were compared after the drawings, both visually and by various different surface test methods. The visual observations already showed that after drawings, the surface of the mechanically cleaned extruded tube had a remarkably higher quality. By applying spectroscopic surface test methods, it was found out the after drawings, in the mechanically cleaned extruded tube the carbon content of the inner surface of the tube end product was only a tenth part of the quantity that is after drawings represented on the inner surfaces of an end product of a regular extruded tube. The results were obtained by comparing the percentage shares of carbon, oxygen and copper on the inner surfaces.

By comparing the above mentioned results with an observation system where the atomic percentage shares of the elements of the inner surface are studied as functions of depth, there is also detected that at a given depth, the mechanically cleaned inner surface contains a remarkably lower degree of carbon than the uncleaned inner surface.

In the end, the tubes under comparison were subjected to a degreasing, pickling and coating treatment. The layer thickness of a metallic coating was larger by about 20%, and the parameter describing the adhesion and integrity of the coating was over 5 times better in the tube that was made of the mechanically cleaned extruded tube. It was also found out that in the case of an uncleaned extruded tube, the graphite-containing drawing grooves on the inner surface were clearly visible in the coating.

Various different methods and visual observations for defining the surface carbon content prove that by using the method according to the invention, there is achieved the best inner surface quality in the end product.

For a man skilled in the art, it is obvious that the different modifications of the invention are not restricted to the above described examples, but may vary within the scope of the appended claims.

## Claims

1. A method for manufacturing copper or copper alloy tube, which method includes an extrusion step and at least one working step in order to work the tube to its final size, and according to which method, the inner surface of the tube is subjected to a cleaning treatment, whereby the cleaning treatment is carried out on the inner surface of the extruded tube in order to remove graphite and carbon based impurities, contaminations and residues and to control the carbon content of the inner surface of the tube before the tube is worked to its final size.

2. A method according to claim 1, **characterized in that** the tube is worked to its final size by drawing the extruded tube at least in one step.

3. A method according to claim 2, **characterized in that** the cleaning treatment is carried out between the extrusion step and the drawing step.

4. A method according to claim 1, **characterized in that** the tube is worked to its final size by rolling the extruded tube at least in one step.

5. A method according to claim 4, **characterized in that** the cleaning treatment is carried out between the extrusion step and the rolling step.

6. A method according to claim 1, 3 or 5, **characterized in that** the cleaning treatment is carried out mechanically.

7. A method according to claim 6, **characterized in that** the cleaning treatment is carried out by treating the inner surface of the extruded tube with a device made of a material that is essentially harder than the inner surface.

8. A method according to claim 7, **characterized in that** the employed cleaning device is a steel brush.

9. A method according to claim 7 or 8, **characterized in that** the cleaning device is moved along the inner surface of the extruded tube by means of magnets.

10. A method according to claim 7 or 8, **characterized in that** the cleaning device is moved along the inner surface of the extruded tube by means of an elongate shaft.

11. A method according to claim 7 or 8, **characterized in that** in the cleaning treatment, the extruded tube is moved with respect to the cleaning device.

12. A method according to claim 6, **characterized in that** the cleaning treatment is carried out by grain blasting, such as sand blasting.

13. A method according to claim 6 - 12, **characterized in that** after the mechanical cleaning treatment, the inner surfaces of the extruded tube are blasted by gas.

14. A method according to claim 6 - 12, **characterized in that** after the mechanical cleaning treatment, the inner surfaces of the extruded tube are washed by liquid.

15. A method according to any of the preceding claims, **characterized in that** the tube is subjected to a coating treatment after working the tube to its final size.

## Patentansprüche

1. Verfahren zum Herstellen eines Kupfer- oder Kupferlegierungsrohres, welches Verfahren einen Extrusionsschritt und mindestens einen Bearbeitungsschritt zum Verarbeiten des Rohres in seine finale Größe aufweist, wobei gemäß dem Verfahren die Innenfläche des Rohres einer Reinigungsbehandlung unterzogen wird, wobei die Reinigungsbehandlung auf der Innenfläche des extrudierten Rohres ausgeführt wird, um Verunreinigungen, Kontaminationen und Restbestandteile basierend auf Grafit und Kohlenstoff zu entfernen, und um den Kohlenstoffgehalt der Innenfläche des Rohres zu kontrollieren, bevor das Rohr in seine letztendliche Größe gebracht wird.

2. Verfahren gemäß Anspruch 1,
**dadurch gekennzeichnet, dass** das Rohr in seine finale Größe mittels Ziehverfahren des extrudierten Rohres in zumindest einem Verfahrensschritt gebracht wird.

3. Verfahren nach Anspruch 2,
**dadurch gekennzeichnet, dass** die Reinigungsbehandlung zwischen dem Extrusionsschritt und dem Ziehschritt ausgeführt wird.

4. Verfahren nach Anspruch 1,
**dadurch gekennzeichnet, dass** das Rohr in seine finale Größe mittels Walzverfahren des extrudierten Rohres in zumindest einem Schritt gebracht wird.

5. Verfahren nach Anspruch 4,
**dadurch gekennzeichnet, dass** die Reinigungsbehandlung zwischen dem Extrusionsschritt und dem Walzschritt ausgeführt wird.

6. Verfahren nach Anspruch 1, 3 oder 5,
**dadurch gekennzeichnet, dass** das Reinigungsverfahren mechanisch ausgeführt wird.

7. Verfahren nach Anspruch 6,
**dadurch gekennzeichnet, dass** die Reinigungsbehandlung ausgeführt wird, indem die Innenfläche des extrudierten Rohres mit einer Vorrichtung behandelt wird, die aus einem Material gefertigt ist, das im Wesentlichen härter ist als die Innenfläche.

8. Verfahren nach Anspruch 7,
**dadurch gekennzeichnet, dass** die eingesetzte Reinigungsvorrichtung eine Stahlbürste ist.

9. Verfahren nach Anspruch 7 oder 8,
**dadurch gekennzeichnet, dass** die Reinigungsvorrichtung entlang der Innenfläche des extrudierten Rohres mittels Magneten bewegt wird.

10. Verfahren nach Anspruch 7 oder 8,
**dadurch gekennzeichnet, dass** die Reinigungsvorrichtung entlang der Innenfläche des extrudierten Rohres mittels einer langgestreckten Welle bewegt wird.

11. Verfahren nach Anspruch 7 oder 8,
**dadurch gekennzeichnet, dass** das extrudierte Rohr bei der Reinigungsbehandlung relativ zur Reinigungsvorrichtung bewegt wird.

12. Verfahren nach Anspruch 6,
**dadurch gekennzeichnet, dass** die Reinigungsbehandlung mittels Korngebläse, wie beispielsweise einem Sandstrahlverfahren ausgeführt wird.

13. Verfahren nach einem der Ansprüche 6 - 12,
**dadurch gekennzeichnet, dass** nachfolgend der mechanischen Reinigungsbehandlung die Innenflächen des extrudierten Rohres mit Gas ausgeblasen werden.

14. Verfahren nach einem der Ansprüche 6 - 12,
**dadurch gekennzeichnet, dass** nachfolgend der mechanischen Behandlung die Innenflächen des extrudierten Rohres mit einer Flüssigkeit gewaschen werden.

15. Verfahren nach einem der vorangehenden Ansprüche,
**dadurch gekennzeichnet, dass** das Rohr einer Beschichtungsbehandlung unterzogen wird, nachdem das Rohr in seine finale Größe gebracht worden ist.

## Revendications

1. Procédé de fabrication d'un tube en cuivre ou en alliage de cuivre, ce procédé comportant une étape d'extrusion et au moins une étape d'usinage destinée à usiner le tube à sa taille finale, et selon lequel procédé la surface intérieure du tube est soumise à un traitement de nettoyage, le traitement de nettoyage étant réalisé sur la surface intérieure du tube extrudé dans le but de retirer les impuretés à base de graphite et de carbone, les contaminations et les résidus et de contrôler la teneur en carbone de la surface intérieure du tube avant que le tube soit usiné à sa taille finale.

2. Procédé selon la revendication 1, **caractérisé par le fait que** le tube est usiné à sa taille finale en étirant le tube extrudé au moins au cours d'une étape.

3. Procédé selon la revendication 2, **caractérisé par le fait que** le traitement de nettoyage est réalisé entre l'étape d'extrusion et l'étape d'étirage.

4. Procédé selon la revendication 1, **caractérisé par le fait que** le tube est usiné à sa taille finale en laminant le tube extrudé au moins au cours d'une étape.

5. Procédé selon la revendication 4, **caractérisé par le fait que** le traitement de nettoyage est réalisé entre l'étape d'extrusion et l'étape de laminage.

6. Procédé selon la revendication 1, 3 ou 5, **caractérisé par le fait que** le traitement de nettoyage est réalisé de façon mécanique.

7. Procédé selon la revendication 6, **caractérisé par le fait que** le traitement de nettoyage est réalisé en traitant la surface intérieure du tube extrudé avec un dispositif constitué d'un matériau plus dur que la surface intérieure.

8. Procédé selon la revendication 7, **caractérisé par le fait que** le dispositif de nettoyage employé est une brosse en acier.

9. Procédé selon la revendication 7 ou 8, **caractérisé par le fait que** le dispositif de nettoyage est déplacé le long de la surface intérieure du tube extrudé au moyen d'aimants.

10. Procédé selon la revendication 7 ou 8, **caractérisé par le fait que** le dispositif de nettoyage est déplacé le long de la surface intérieure du tube extrudé au moyen d'une tige allongée.

11. Procédé selon la revendication 7 ou 8, **caractérisé par le fait que**, dans le traitement de nettoyage, le tube extrudé est déplacé par rapport au dispositif de nettoyage.

12. Procédé selon la revendication 6, **caractérisé par le fait que** le traitement de nettoyage est réalisé par grenaillage, tel que le sablage.

13. Procédé selon les revendications 6 à 12, **caractérisé par le fait que**, après le traitement de nettoyage mécanique, du gaz est projeté sur les surfaces intérieures du tube extrudé.

14. Procédé selon les revendications 6 à 12, **caractérisé par le fait que**, après le traitement de nettoyage mécanique, les surfaces intérieures du tube extrudé sont rincées avec du liquide.

15. Procédé selon l'une quelconque des revendications précédentes, **caractérisé par le fait que** le tube est soumis à un traitement de revêtement après l'usinage du tube à sa taille finale.
